

## UNITED STATES PATENT OFFICE

2,138,325

## PROCESS OF MAKING NEUTRAL SIZED PAPER

Walter A. Nivling, Newton Center, Mass.

No Drawing. Application March 26, 1936,  
Serial No. 71,058

5 Claims. (Cl. 92—40)

One object of this invention is to set forth methods and materials which will produce a well-sized paper not only on both surfaces but throughout the sheet so that the inner portions are also so substantially sized as to permit satisfactory writing with pen and ink even following erasure. A further object is to produce a paper free from acidity thereby assuring greater strength and permanency.

10 The advantage of resistance to the penetration of ink or water and particularly to hot water long enough to adequately meet commercial or industrial requirements is obvious.

The present commercial method of obtaining 15 the desired degree of resistance to ink or water is to add from one to five per cent of a solution or emulsion of rosin soap to the paper fibers while they are suspended in from twenty to two hundred times their weight of water. This addition 20 of rosin soap is followed or preceded by the addition of alum. The amount of alum required varies from an equal to two to three times the weight of the rosin used. Rosin soap (sodium to 25 resinate) reacts chemically with the alum to form an aluminum resin complex commonly described as aluminum resinate. This aluminum resinate is water repellent and when deposited on the paper fibers or mechanically interlocked among the paper fibers gives to the finished 30 paper the desired ink or water resistance.

The obtaining of the desired degree of ink or water resistance consistently is one of the greatest problems of the paper manufacturer. Difficulty in obtaining satisfactory ink or water 35 resistance commonly described as "sizing", arises from various interfering substances and conditions. For example, hard waters containing calcium or magnesium, or returned white waters gradually building up excessive amounts of 40 sodium sulphates, interfere with the formation of the desired ink or water resistant aluminum resinate. High temperatures existing in intake water or built up by prolonged beating greatly increase the difficulty of obtaining satisfactory 45 ink or water resistant sizing. High pH or alkalinity of the water in which the fibers are suspended greatly interferes with proper sizing. Other factors make ink or water resistant sizing of the fibers while they are in suspension difficult. Even very active agitation such as Jor- 50 daning reduces and at times destroys the effectiveness of rosin sizing if this be done prior or incident to the Jor daning operation.

Another improvement in the quality of paper 55 not possible by methods now employed but made

possible by my new method which I will describe hereafter is that of correcting two-sidedness of paper. Two-sidedness is an inherent quality of all papers whether these papers are sized or not. This two-sidedness is due in part at least to existing methods of making paper, particularly by the use of the Fourdrinier wire. In the Fourdrinier wire method of forming the sheet of paper, the paper making fibers in suspension in approximately two hundred times their weight 10 of water are flowed onto a moving screen wire through which the water drains, aided first by the vibration of the wire and later by the aid of suction boxes and sometimes with the further aid of a suction couch roll. In this removal of the 15 water, there is also removed some of the finer fibers and other suspended matter from the side of the paper adjacent to the wire. Obviously, the top side of the sheet is more compact because the paper fibers already deposited form a screen 20 or mat which retains and thus makes the top surface more dense in comparison with the wire surface of the sheet. This inherent two-sidedness results in not only a less dense sheet but also a less well-sized sheet on the wire side. 25 When paper fibers are dyed in the beaters and then formed on the wire, this two-sidedness is immediately apparent to the eye when the top side and reverse side are brought into the same plane of view. Obviously two-sidedness is most 30 noticeable on a colored or filled sheet. This two-sided sheet when dried and submitted to surface sizing consequently absorbs the surface sizing more on one side than on the other. This further augments the differences due to two-sidedness. "Curl" and "buckle" are largely due to two-sidedness which affects the rate of moisture absorption when the finished paper is exposed to an atmosphere of higher or lower humidity as in the 35 print shop. This is the cause of many complaints and losses to the paper maker. 40

By the new process described herein the difficulties due to two-sidedness are largely overcome. The two-sidedness is corrected by a 45 double application of my new sizing solution which combines both water or ink resistant sizing and surface sizing. Obviously, if in the first sizing step in my new process there still remains some two-sidedness due to the inherent difference in the formation of the two sides, this 50 is corrected by the second application of my new sizing. Since the first application produces a very measurable degree of water and ink resistance, and since this degree of water and ink resistance or coloring is different on the two sides, 55

it follows that there will be a difference in the absorption of the second application thus equalizing and overcoming the difference existing before. This is quite impossible with the present 5 method of sizing. This point becomes distinctly noticeable if the dyeing and sizing are applied simultaneously. The first application may still show a difference in the degree of coloring but when the second application is made owing to a 10 difference in absorption due to the two-sidedness, the amount absorbed is reversed and both sides will then show the same depth of color shade. For the same reason, the amount of size on the two sides will be the same thus greatly reducing 15 the tendency to curl and buckle. This will be apparent to anyone skilled in the art of paper making.

To overcome these various difficulties and others such as foaming, foam spots, pitch troubles, 20 choking of screen wires and felts, etc., my plan provides for the forming of the desired aluminum resinate in a vat separate from that in which the fibers are suspended and adding this aluminum resinate to the fibers after they have been substantially 25 formed into their final position and after approximately eighty-five to ninety per cent or more of the water in which the fibers were previously suspended has been removed. To do this and obtain satisfactory ink or water 30 resistant sizing and a paper free from harmful acidity which results from the chemical interaction between rosin soap and alum as now used, it is essential that the aluminum resinate or its equivalent shall be formed and retained 35 in a colloidally fine state of sub-division so that it may properly penetrate and deposit on all the fiber faces and interfaces. It is also essential that the by-product acidity be neutralized. While various methods of applying sizing to the 40 paper web after it has been at least partially formed have previously been proposed, none of them as far as I am aware have produced satisfactorily sized paper and none of them have solved the problems of two-sidedness or of correcting the acidity of the fibers.

For the purpose of describing this invention, when the term "colloidal solutions" or "colloidal suspensions" is employed, it will suffice to describe "colloidal solutions" or "colloidal suspensions" as those in which the substances dissolved or suspended are of sufficiently small particle size to permit light to pass through or between the particles to such an extent as will permit type to be read through a half-inch depth of the 50 liquid, cooled to room temperature and aged for from two or four hours or more. This bespeaks a particle size sufficiently small to permit free penetration into the pores of the papers commercially known as newsprint paper, wrapping 55 paper, writing paper, including bonds and ledger papers.

Colloidal dispersions of aluminum resinate as above described can then be added to the web of paper or other paper articles and will penetrate freely. The water coincidentally added may be removed by any of the usual drying processes. The application of colloidally fine aluminum resinate may be made by adding to the fibers while they are suspended in water in 60 the beaters or at the head box or other intermediate point since the aluminum resinate particles are attracted to and held by the fibers. It is preferable, however, to add the suspension of aluminum resinate either on the wire at the 65 suction couch roll or at the dandy roll since if

added at either of these points ninety percent of the water previously used will have been removed with the advantage of attaining greater economy and avoiding difficulties incident to sizing in the presence of a large excess of water. 5 The application may also be made at the press rolls or any desired point along the bank of driers, or if desired, the application may be made as that of the usual surface sizing procedure. It is preferable in many cases particularly with 10 very light papers, to give some preliminary sizing in the beaters, so that when the size is applied to the web there will not be too great absorption, which would result in weakening the web or undesirably adding to the drying operation. For this preliminary sizing it is preferable 15 to follow what is one standard practice, that is, to add the rosin to the pulp first and then to precipitate it with alum, taking care that an excess of the latter be not used. 20

One way of making the desired colloidally, finely divided aluminum resinate is to dissolve the rosin soap (sodium resinate plus free unsaponified resin) together with a suitable protective colloid in water in such proportions so 25 that there will be from one-quarter to three per cent of resin and from one to ten per cent of the protective colloid present. In these varying proportions it is desirable to correlate the amount 30 of colloid to rosin so that the protective colloid will not be present in more than five times the amount of original rosin which enters into the sizing compound. The solution so prepared is 35 mixed with an equal volume of a solution containing a like amount of the protective colloid together with a soluble aluminum salt such as for example papermakers alum. The amount of alum or other soluble aluminum salt may vary from one-half to twice or more times the dry 40 weight of the rosin soap used. 40

By the term "protective colloid", I mean that of the many substances known as "colloids", choice shall be made of such as will effectively prevent the reaction product, aluminum resinate, 45 from aggregating into large particle size, generally described as "flocs".

Several materials may be used as protective colloids such as, for example, animal glue, gum arabic, casein or soluble starch. I have found the widely used soluble starch gum material 50 known in the trade as "Hercules Gum" well suited for serving as a protective colloid.

When the two solutions, one containing the rosin soap together with the protective colloid; the other containing the alum together with the 55 protective colloid, are mixed, the chemical interaction forming the aluminum resinate takes place in whole or in part and more aluminum resinate is formed during the drying process. It is almost universally found necessary to use 60 more than the theoretical amount of alum or other aluminum salt to dissociate the sodium resinate. This excess alum ionizes, forming an acid state. This acidity weakens the paper fiber not only during the process of paper making but 65 continuing after the paper has been dried with destructive effect on the strength and folding quality of the paper.

To overcome this undesirable acidity, various alkaline reacting substances have been proposed 70 to neutralize the acidity, such as caustic soda, soda ash, bicarbonate of soda, borax, sodium aluminate, triethanolamine and others. Paper manufacturers have used these various alkalies but their use is attended with great danger 75

since, if such an amount of any of the alkalies above mentioned is used as will neutralize the acidity, a secondary reaction takes place whereby at least part of the aluminum resinate is decomposed with more or less complete sacrifice of the desired ink or water resistant sizing.

After much investigation, I have found that if ammonium hydrate is used in the presence of a suitable colloid not only can enough be used 10 to completely neutralize the free acidity but even a marked excess may be used with the result that harmful acidity is overcome without the destruction of the aluminum resinate. In fact, I have found that several times the amount of ammonium hydrate necessary to neutralize the acidity 15 may be used, if in the presence of a suitable colloid, without any harmful effect on or decomposition of the ink or water resistant aluminum resinate. This has the great advantage of 20 permitting the addition of a satisfactory neutralizing alkali without requiring the attendance of a chemist since by a simple testing with suitable indicators or even by the slight odor of ammonia, the man in the mill can produce the desired result without fear of harmful excess since an 25 excess of ammonium hydrate will be evaporated during the drying and the finished paper will be quite neutral. This has long been desired for all paper and more particularly for permanent 30 record papers. The amount of ammonium hydroxide can be more accurately determined by the usual methods of determining the hydrogen ion concentration, the measure of which is commonly referred to as the pH value. Provided the 35 pH value of the sizing bath is at least 6.5 there will be sufficient ammonia for the purpose, although it is preferred to maintain the pH slightly higher than this in order to insure against loss of ammonia by evaporation and to neutralize 40 harmful residual acidity of the fibers.

The ammonia not only neutralizes the acidity of the paper web, but also acts to preserve the sizing dispersion in the colloidal condition best suited for use. It is well known that surface 45 sizing baths become less efficient upon prolonged contact with the paper fibers, probably due to the taking up of acids from the paper fibers, and the use of ammonia as above described has proved to be advantageous in maintaining the bath in 50 effective condition.

It will be apparent to anyone skilled in the art that the materials used may be replaced by equivalents and that the proportions above mentioned are typical only. Aluminum acetate or 55 various alums or other aluminum salts may replace paper makers alum; sodium stearate may replace sodium resinate; ammonium resinate may replace sodium resinate; other colloids may replace the soluble starch "Hercules"; the ammonium hydrate may be replaced by another volatile alkali; and the particular method outlined 60 for making and blending the reacting chemicals and colloids may be changed, and the proportions may be changed as may be more convenient or 65 found best suited for the particular type of paper being made. Dyestuffs may be added to color the paper as part of the process described above and either or both the sizing and the coloring may be done in several stages as, for example, 70 part may be added while the paper making fibers are in a free flowing state of suspension, and a subsequent sizing and/or coloring may be made at any convenient point during the drying or 75 the paper may be dried and subsequently sized and/or sized and colored in one or two steps as

may be found most convenient or desirable, without departing from the spirit of my invention.

My claims on which I desire to secure Letters Patent are:

1. A process of sizing a paper web which comprises subjecting the formed and at least partially dried web to an aqueous sizing bath consisting of the reaction product of one-eighth to one and a half percent of rosin soap and paper makers alum in an amount equal to one half 10 to twice the amount of rosin soap, one to ten percent of a protective colloid, there being not more than ten times the amount of protective colloid as rosin, and ammonium hydroxide in sufficient amount to maintain a substantially 15 non-acid reaction in that portion of the bath in contact with the fibers throughout such period of contact, and thereafter drying the web to remove water and excess ammonia and to produce a substantially neutral dried web. 20

2. In a process of obtaining a sized, substantially neutral web, the steps comprising subjecting the web forming fibers to the action of an aqueous bath containing a colloidal dispersion of aluminum resinate, a protective colloid, and ammonium hydroxide in sufficient amount to preserve in that portion of the bath in contact with the fibers a pH of at least 6.5 throughout such period of contact, and thereafter drying the web to remove water and excess ammonia and to produce a substantially neutral dried web. 25

3. In a process of obtaining a sized web free from the harmful acidity resulting from rosin sizing, the steps comprising subjecting the web forming fibers to the action of an aqueous bath 35 containing a colloidal dispersion of the reaction product of sodium resinate and alum, a protective colloid, and ammonium hydroxide in sufficient amount to maintain a non-acid reaction in that portion of the bath in contact with the fibers throughout such period of contact, and thereafter drying the web to remove water and excess ammonia and to produce a substantially neutral dried web. 40

4. In a process of obtaining a sized, substantially neutral paper web substantially free from two-sidedness, the steps comprising subjecting the paper forming fibers to the action of an aqueous bath containing a colloidal dispersion of the reaction product of rosin soap and alum, 50 a protective colloid, and ammonium hydroxide in sufficient amount to maintain a non-acid reaction in that portion of the bath in contact with the fibers throughout such period of contact, at least partially drying the web, subjecting both sides of the web a second time to the action of another aqueous bath containing a colloidal dispersion of the reaction product of rosin soap and alum, and thereafter drying the web to remove water and excess ammonia and 60 to produce a substantially neutral web. 55

5. In a process of obtaining a sized paper web substantially free from acidity which comprises forming the fibers into at least partial web form, subjecting the fibers of the web thus formed to 65 the action of an aqueous bath containing a colloidal dispersion of aluminum resinate, a protective colloid, and ammonium hydroxide in sufficient amount to maintain in that portion of the bath in contact with the fibers a pH of at least 6.5 70 throughout such period of contact, and thereafter drying the web to remove water and excess ammonia. 75